

# UNITED STATES PATENT OFFICE.

CHARLES MORRIS JOHNSON, OF AVALON, PENNSYLVANIA.

## ALLOY STEEL.

1,420,707.

Specification of Letters Patent. Patented June 27, 1922.

No Drawing.

Application filed August 6, 1920. Serial No. 401,656.

To all whom it may concern:

Be it known that I, CHARLES MORRIS JOHNSON, residing at Avalon, in the county of Allegheny and State of Pennsylvania, a citizen of the United States, have invented or discovered certain new and useful Improvements in Alloy Steel, of which improvements the following is a specification.

I have discovered a new alloy steel, the composition of which may be varied within limits to be hereinafter defined, which possesses to a marked degree many highly desirable physical properties. It is non-magnetic. It is strongly resistant to scaling by heat, and to the action even of the oxyacetylene flame. It resists rust, as well as attack by acids. It is also non-brittle, but is tough and highly ductile, while sufficiently hard for a great variety of uses.

This new alloy steel is a chromium-nickel-silicon steel, containing not less than ten per cent of chromium, not less than nine per cent of nickel, and not less than one per cent of silicon. The chromium should not exceed twenty per cent, the nickel twenty-five per cent, or the silicon ten per cent. The chromium and nickel are advantageously used in substantially equal proportions, though this is subject to some variation.

For instance in some cases I have used 16 per cent chromium with 10 per cent nickel and 1.50 per cent silicon, and in other cases 16 per cent chromium with 18 or 20 per cent nickel and 3 per cent silicon. For most purposes I prefer to use between fifteen and twenty per cent each of nickel and chromium and from three to four per cent silicon. Though higher carbon may be used for particular purposes, the carbon content should not ordinarily exceed one per cent, and for most purposes I prefer to keep the carbon below .40 per cent.

When tested in comparison with other steels considered as resistant as any so far known, by immersion for 24 hours in both dilute sulphuric acid and dilute hydrochloric acid, the steels of the compositions

above stated were much more lightly attacked, indeed hardly attacked at all. The steel is also highly resistant to dilute nitric acid (32% acid). In still other tests in water, while the other so-called non-corrosive steels were badly rusted, my steel was only slightly stained at the water level, without any progressive rusting at all. 55

My steel cannot be burned, that is to say, rendered crystalline and brittle, at a temperature as high as 2400° F. In fact after having been exposed to that temperature, tests showed its elongation and its reduction in area to be each 67 per cent. It is consequently very workable hot, and it can be formed cold into many varieties of vessels and utensils in which its resistant properties are desirable. Being also of high tensile strength 65 it may be used for boiler-tubes, cutlery, engine parts in internal combustion engines, and dies for die casting. And it may be used generally for purposes where toughness, or resistance to heat or corrosion are 70 required.

It is a matter of common experience that nickel and cobalt have many like chemical properties, and that their metallurgical effects in alloy steels are generally alike, so 75 I desire it to be understood that in the appended claim I intend to cover the use of cobalt as a substitute for nickel in whole or in part. The steel may of course contain the usual small quantities of manganese, etc., 80 and other alloying elements may also be employed without departure from the invention.

I claim as my invention:

Steel containing from about ten per cent to about twenty per cent of chromium, from 85 about nine per cent to about twenty-five per cent of nickel, and from about one per cent to about ten per cent of silicon.

In testimony whereof I have hereunto set my hand.

CHARLES MORRIS JOHNSON.

Witnesses:

G. G. TRILL,  
MARSHALL A. CHRISTY.